

M. O. SEM.

PROCESS OF PRECIPITATING ALUMINIUM COMPOUNDS.

APPLICATION FILED APR. 23, 1918.

1,382,808.

Patented June 28, 1921.



Inventor,  
Mathias Ovrom Sem

By *Dorsey & Cole*  
Attorneys

# UNITED STATES PATENT OFFICE.

MATHIAS OVROM SEM, OF CHRISTIANIA, NORWAY, ASSIGNOR TO DET NORSKE AKTIESELSKAB FOR ELEKTROKEMISK INDUSTRI, OF CHRISTIANIA, NORWAY.

## PROCESS OF PRECIPITATING ALUMINIUM COMPOUND.

1,382,808.

Specification of Letters Patent. Patented June 28, 1921.

Application filed April 23, 1918. Serial No. 230,250.

To all whom it may concern:

Be it known that I, MATHIAS OVROM SEM, a subject of Norway, and a resident of Christiania, Kingdom of Norway, have invented 5 certain new and useful Improvements in Processes of Precipitating Aluminium Compounds, of which the following is a specification.

This invention relates to the manufacture 10 of aluminium compounds and has for its object a process whereby such compounds can be manufactured on a commercial scale by means of electrolysis.

It has hitherto been impracticable to produce 15 aluminium compounds in an economical way, from solutions obtained by decomposition of minerals containing aluminium by means of acid. Decomposition by means of an alkali is generally used in the production 20 of aluminium compounds.

I have however found a simple method for precipitating aluminium compounds from solutions containing aluminium combined 25 with a mineral acid. I cause a precipitation of aluminium compounds by means of electrolysis. The electrolysis is preferably carried out in a suitable vessel divided into anode and cathode compartments by a porous diaphragm. Preferably an insoluble 30 anode is employed and a small amount of alkali salts is added to the electrolyte.

When electrolysis is started aluminium 35 hydrate, or in a sulfate solution basic aluminium sulfate containing varying amounts of  $\text{SO}_4$  will precipitate at the cathode.

In neutral solutions which in themselves 40 have no oxidizing effect the precipitate obtained will be practically free from iron for the known reason that ferrous iron will not precipitate as long as an excess of aluminium compounds is present in the solution, and because of the hydrogen evolved at the 45 cathode ferric iron originally present will be reduced and kept in the ferrous state or precipitated on the cathode as metallic iron. On account of their low content of iron, aluminium compounds precipitated as above described are very well adapted for the manufacture of aluminium and for similar purposes where a great purity is required.

If a nitric acid solution is used in the electrolysis the reduction taking place at the cathode will result in the formation of ammonia from nitric acid. The ammonia will

immediately precipitate a corresponding 55 amount of aluminium hydrate, being itself converted to a nitrate, and thus increase the output directly due to electrolysis.

The acid liberated at the anode by the electrolysis may be utilized in various manners. I may subject such acid to a concentration process and use it for the decomposition 60 of new amounts of raw material. But I have found that if the raw material used is fairly easily soluble as is the case with bauxite and 65 some silicates such as labradorite, I can suspend the raw material in the anode compartment and it will then become dissolved as soon as sufficient acid is liberated, without special concentration of the acid. 70

As the raw materials used always contain other soluble compounds than aluminium compounds, these will combine with an equivalent amount of the acid used and must from time to time be removed from the 75 process in the form of salts. In this case an amount of acid corresponding to that removed in the form of salts must be added to the process.

I have found that my above described 80 method may be carried out continuously and that it is especially suited for minerals of the series labradorite-anorthosite and other minerals rich in anorthite, as these minerals may be directly decomposed by means of the 85 acid formed during the electrolysis. I prefer to carry out the treatment in a sulfate solution, but it is to be understood that other salts of strong mineral acids may also be used. 90

When the raw material contains soluble bases which will not be precipitated on the cathode, such as for instance alkali metals, more aluminium hydrate will be precipitated 95 at the cathode than will migrate from the anode compartment to the cathode compartment. Therefore aluminium must be supplied to the cathode compartment by other means. Also from time to time the undissolved residue from the raw material must 100 be removed from the anode compartment.

In the following specific example, I will illustrate the preferred way of carrying out my process by using a sulfuric acid solution, reference being had to the accompanying 105 drawing forming part of this application and diagrammatically illustrating an electrolytic vat in vertical section, but it is

understood that my invention is not limited thereto, as the details of my process may vary within wide limits.

A solution containing 70 grams of 5  $\text{Al}_2\text{O}_3$  in the form of  $\text{Al}_2(\text{SO}_4)_3$  and 10 grams of  $\text{Na}_2\text{O}$  in the form of  $\text{Na}_2\text{SO}_4$  per liter is poured into an electrolytic tank A. The cathode compartment F of this tank is separated from the anode compartment G 10 containing an insoluble anode D by means of a diaphragm B of the type ordinarily used for such purposes, cocks H and I being provided to withdraw the contents of the compartments. The temperature of the solution is preferably kept at 60-80° C. When 15 electric current is supplied the voltage between anode and cathode will be about 5 volts. During electrolysis a precipitation will take place near the cathode E and at 20 the same time the iron in the solution will be deposited on the cathode. The precipitation consists of aluminium hydrate containing small amounts of  $\text{SO}_3$  in the form of 25 adsorbed acid or a basic sulfate and is removed from the solution from time to time, subjected to washing and if pure  $\text{Al}_2\text{O}_3$  is desired is calcined, whereby the  $\text{SO}_3$  is eliminated. The calcined product will contain less than 0.1%  $\text{Fe}_2\text{O}_3$  and is very well adapted 30 for the manufacture of aluminium.

In the anode compartment free sulfuric acid is formed. This acid serves to dissolve the raw material, in this case pulverized labradorite, which is continuously added to 35 the anode compartment, dissolution of the raw material being facilitated by agitation.

When a considerable amount of undissolved residue has accumulated in the anode compartment electrolysis is interrupted. 40 The anolyte is separated from undissolved residue by means of filtration and the residue, principally consisting of  $\text{SiO}_2$ , is rejected, the filtrate being returned to the process but being in part poured into the 45 cathode and part into the anode compartment.

At the same time a part of the catholyte is removed and subjected to crystallization in order to remove the salts which accumulate 50 late in the solution. These are principally alkali salts, as the calcium present in the raw material remains in the anode compartment in the form of calcium sulfate, and crystallize out together with aluminium sulfate giving alum as a by-product.

The solution removed from the cathode compartment for crystallization is replaced by a corresponding amount of the filtrate obtained from the anolyte.

60 The anode compartment is then supplied with sulfuric acid of such a strength that the  $\text{H}_2\text{SO}_4$  contained therein will replace the  $\text{H}_2\text{SO}_4$  removed from the catholyte in the form of salts. The electrolysis is then continued as before.

The foregoing detailed description has been given for clearness of understanding and no undue limitation should be deduced therefrom, but the appended claims should be construed as broadly as permissible in view of the prior art.

What I claim as new and desire to secure by Letters Patent of the United States is:

1. In the recovery of aluminium compounds, the process which comprises effecting precipitation thereby subjecting a solution containing an aluminium mineral acid salt to electrolysis and thereby effecting precipitation of an aluminium compound at the cathode. 75

2. In the recovery of aluminium compounds, the process which comprises effecting precipitation thereof by subjecting a solution containing an aluminium sulfate to electrolysis and thereby effecting precipitation of a basic aluminium sulfate at the cathode. 85

3. In the recovery of aluminium compounds, the process which comprises effecting precipitation thereof by subjecting a solution containing an aluminium mineral acid salt to electrolysis in the presence of an alkali salt and thereby effecting precipitation of an aluminium compound at the cathode. 90

4. In the recovery of aluminium compounds, the process which comprises effecting precipitation thereof by subjecting a solution containing an aluminium mineral acid salt to electrolysis in a diaphragm cell and thereby effecting precipitation of an aluminium compound at the cathode. 100

5. In the recovery of aluminium compounds, the process which comprises effecting precipitation thereof by subjecting a solution containing an aluminium sulfate to electrolysis in a diaphragm cell and thereby effecting precipitation of a basic aluminium sulfate at the cathode. 105

6. In the recovery of aluminium compounds, the process which comprises effecting precipitation thereof by subjecting a solution containing an aluminium mineral acid salt in the presence of an alkali salt to electrolysis in a diaphragm cell and thereby effecting precipitation of an aluminium compound at the cathode. 110

7. In the recovery of aluminium compounds, the process which comprises effecting precipitation by subjecting a solution containing an aluminium mineral acid salt to electrolysis in a diaphragm cell having an insoluble anode, and thereby effecting precipitation of an aluminium compound at the cathode. 120

8. In the recovery of aluminium compounds, the continuous process which comprises effecting precipitation thereof by subjecting a solution containing an aluminium mineral acid salt to electrolysis in a dia- 130

phragm cell and thereby effecting precipitation of an aluminium compound at the cathode and liberation of the mineral acid at the anode, and dissolving at the anode by the liberated acid a substance containing combined aluminium.

5 9. In the recovery of aluminium compounds, the continuous process which comprises effecting precipitation thereof by subjecting a solution containing aluminium sulfate to electrolysis in a diaphragm cell and thereby effecting precipitation of a basic aluminium sulfate at the cathode and liberation of sulfuric acid at the anode, and dissolving at the anode by the liberated sulfuric acid a substance containing combined aluminium.

10 10. In the recovery of aluminium compounds, the continuous process which comprises effecting precipitation thereof by subjecting a solution containing an aluminium mineral acid salt in the presence of an alkali

salt to electrolysis in a diaphragm cell and thereby effecting precipitation of an aluminium compound at the cathode and liberation of the mineral acid at the anode, and dissolving at the anode by the liberated acid a substance containing combined aluminium.

11 11. In the recovery of aluminium compounds, the process which consists in making a solution of aluminium salt by subjecting a mineral containing combined aluminium to the action of a mineral acid, subjecting the solution so formed with the addition thereto of an alkali salt to electrolysis in a diaphragm cell having an insoluble anode, thereby effecting precipitation of aluminium compound at the cathode and liberation of the mineral acid at the anode, and dissolving at the anode by the liberated acid more of said mineral.

Signed at Christiania, Norway, this 7th day of March, 1918.

MATHIAS OVROM SEM.